

1

3,127,350

**WHITE OIL STABILIZER**

Oliver C. Kerfoot, New Orleans, La., and Irwin R. Supernaw, Shawnee, Okla., assignors to Continental Oil Company, Ponca City, Okla., a corporation of Delaware  
No Drawing. Filed May 23, 1960, Ser. No. 31,222  
3 Claims. (Cl. 252—35)

This invention relates to improved hydrocarbon oil compositions. More particularly, this invention relates to white mineral oils containing a small amount of homogeneously dispersed zinc 2-ethylhexoate capable of beneficially inhibiting the development of odor and haze normally occurring upon exposure of the oil to sunlight.

The oils contemplated as most suitable for use in accordance with our invention are generally known as highly refined, industrial type white mineral oils and are available commercially in various grades differing chiefly with respect to viscosity properties. When initially produced from their source, namely, crude oil stocks, they are transparent, colorless and substantially odorless oily liquids. Either paraffin-base crudes, naphthene-base crudes or mixtures of said crudes may be employed in obtaining the white mineral oil. Although the quality of the finished product depends primarily upon the degree of care and skill employed in the refining process, certain of its basic properties are determined by the type of crude used. For example, a naphthene-base crude provides a white mineral oil of relatively high specific gravity and viscosity characteristics. On the other hand, a Pennsylvania type paraffin-base crude yields a white oil of generally lower viscosity properties and specific gravity. In addition to the physical properties noted for the various mineral oils derived from the particular sources mentioned, these crudes also yield oils differing somewhat in other properties. For example, white oils derived from paraffin-base crudes exhibit excellent heat resistance and are noted for their affinity for certain waxes. Particularly because of the latter mentioned attribute, an oil of this type is favored in certain applications such as for example in the preparation of cosmetic formulations.

The first step in the production of white oil consists in the removal of the lighter portions of the crude such as gasoline, naphtha, kerosene and certain like fractions such as for example fuel oils. This segregation of the enumerated fractions is customarily accomplished by a heat process referred to as fractional distillation. After the lighter fractions of the crude have been separated as indicated, the oil residue is further distilled. The lower boiling fractions of said residue serve as the raw oil from which the white oils are ultimately obtained via a refining operation.

The primary purpose in refining the raw oil fractions is to remove various reactive and unsaturated hydrocarbons and impurities therefrom, which components are responsible for the color, odor, taste and other objectionable properties normally associated with the unrefined oil. Although the specific details of the refining procedure may vary considerably among the individual manufacturers of the white oil, it will almost always include treatment of the oil with sulfuric acid, washing with alkalies and solvents, and the application of adsorbents.

The purpose of the sulfuric acid treatment is to remove all of the unsaturated, aromatic and other reactive hydrocarbons and most of the impurities that are present in the oil. The action of the treating acid is both chemical and a physical one. In its chemical role, the sulfuric acid reacts with a large proportion of the objectionable components present to yield complexes capable of ready removal. The acid additionally serves as a solvent for

2

the said reaction products or complexes and also effects removal of resinous and asphaltic substances and other like impurities from the oil.

In most of the refining practices the oil is treated with large quantities of either concentrated or fuming sulfuric acid (oleum). The quantity and concentration of acid used, the temperature, the length of treatment and the method of application depends upon the type of crude used and the type of oil and degree of refinement required. Ordinarily, 30 to 70% of acid based on the weight of the oil is used. The contact time of acid with oil varies extensively as indicated and ranges from as brief as a few minutes in continuous treating to about one hour in batch processes.

Following the acid treatment, the oil is usually further refined by some sort of adsorption process in order to remove minute traces of carbon, coke, resinous and asphaltic substances, coloring matter, moisture, etc. The commonly used adsorbents are of mineral origin and include fuller's earths in natural state or in acid-activated form, e.g., bauxite, bentonite, etc. Adsorbents of organic origin such as charcoal, activated carbon and the like as well as such substances as silica gel, alumina gel or similar synthetic adsorbents are also used.

White mineral oils are employed in a legion of industrial applications. The particular application involved more or less dictates the grade of mineral oil to be used, especially as regards its viscosity characteristics. Accordingly, one can find numerous commercial products generally sold to meet relatively narrow viscosity specifications. Thus one may readily avail of proprietary products ranging in viscosity from as low as 30 SSU units Saybolt at 100° F. to a viscosity of as high 500 SSU. Of this broad range of viscosities that may be found in products of this type, there are two general classifications, namely, light viscosity or simply light white mineral oils, i.e., those having a Saybolt viscosity of not more than about 170 SSU at 100° F. and heavy white mineral oils which have higher viscosity than that specifically stated.

Details with respect to the aforesaid viscosity characterization of oil products may be found in ASTM test D445—46T.

Apart from lubricating applications which usually include most lubricants for food processing apparatus wherein a medicinal grade of oil is required, there are many other type applications in which a so-called technical grade of white mineral oil is perfectly satisfactory. The technical grade designation connotes an oil which is highly refined and substantially chemically inert, but not so absolutely inert as to permit use for medicinal purposes as an internal lubricant. The technical grade oils are used extensively in cotton processing, leather dressings, and especially in the preparation of cosmetics or cosmetic bases, such as makeup preparations, cold creams, hair preparations and the like. Our invention especially pertains to technical grade white mineral oils useful in the latter applications among others of a similar nature.

It is known that all white mineral oils, however fully refined, have a tendency to deteriorate with a development of haze and odor which development is greatly accelerated upon exposure of the oil to light, particularly at elevated temperatures. The odor experienced is that of a disagreeable hydrogen sulfide odor and although while the amounts of hydrogen sulfide generated in such a deterioration process are extremely small they are nevertheless perceptibly obnoxious.

We have found that when the substance zinc 2-ethylhexoate is added to refined white mineral oils in relatively minute quantities, the oil is inhibited towards the formation of hydrogen sulfide and haze development. As mentioned previously, the deterioration or formation of hy-

hydrogen sulfide and haziness is known to be contributed to and aggravated by exposure of the oil to actinic radiation. Accordingly, it was most surprising to find that zinc 2-ethylhexoate when contained in a white mineral oil in the contemplated minute quantities has the ability to effectively adsorb ultraviolet light; for this appears to be the process by which the degenerative effects of the incident actinic light are principally thwarted. Nevertheless, we believe that the function of the zinc soap extends beyond mere ultraviolet light adsorption because we have employed substituted benzophenone light adsorbers exhibiting high ultraviolet adsorption characteristics and have found that they were not nearly as effective in retarding deterioration of the white mineral oil as our stabilizer.

The zinc soap useful in the practice of our invention is admirably adapted for the purposes intended because the compound itself is odorless, substantially colorless, practically nontoxic, readily soluble in the white oil and at the same time considerably more stable toward oxidation and deterioration upon aging and exposure to light and heat than the white oil itself which obviously is a fundamental prerequisite for an inhibitor of this type.

The amount of zinc 2-ethylhexoate that can be added to the white mineral oil in order to achieve effective protection ranges from as low as 50 p.p.m. based on the oil. The preferred range of the additive extends from about 100 to 1000 p.p.m. Amounts greater than 1000 p.p.m. can be used but the extent of improvement in stabilization to be realized in using these higher amounts is not economically warranted.

Incorporation of the zinc soap into the white oil poses no problem and it can be incorporated therein by moderate stirring of the two components, shaking, etc.

In order to further illustrate the nature of this invention, the following example is given in which all parts are parts by weight. This example is not to be construed as limitative of the invention since the only limitations intended are those expressed in the appended claims.

#### EXAMPLE I

Into portions of a white mineral oil having a Saybolt viscosity of 70 SSU at 100° F. was added zinc 2-ethylhexoate (22% zinc content) in concentrations ranging from 125 to 1000 p.p.m. based on the weight of the oil.

The samples were stirred in order to effect solution of the zinc soap in the oil and then exposed in the glass bottles to direct sunlight for a number of days along with an untreated sample of the same oil. The samples were observed for development of hydrogen sulfide and haze at daily intervals. The results of these experiments are tabulated in Table I below.

Table I

| 10 | Sample | Concentration of Additive in oil in p.p.m. | Results of Exposure Test                            |
|----|--------|--------------------------------------------|-----------------------------------------------------|
| 15 | A----- | 0                                          | Heavy H <sub>2</sub> S and haze in about 4-6 hours. |
|    | B----- | 125                                        | H <sub>2</sub> S in 2 days—No haze.                 |
|    | C----- | 250                                        | H <sub>2</sub> S in 3 days—No haze.                 |
|    | D----- | 500                                        | H <sub>2</sub> S in 4 days—No haze.                 |
|    | E----- | 1,000                                      | No H <sub>2</sub> S or haze after 5 days.           |

20

What is claimed is:

1. A composition of matter consisting essentially of a colorless and odorless white mineral oil free of unsaturated and aromatic hydrocarbons containing from about 0.005% to 0.1% of zinc 2-ethylhexoate.

2. A composition of matter consisting essentially of a colorless and odorless white mineral oil free of unsaturated and aromatic hydrocarbons having a Saybolt viscosity of less than about 170 SSU at 100° F. containing from about 0.005% to 0.1% of zinc 2-ethylhexoate.

3. A composition of matter consisting essentially of a colorless and odorless white mineral oil free of unsaturated and aromatic hydrocarbons having a Saybolt viscosity of about 70 SSU at 100° F. containing from about 0.005% to 0.1% of zinc 2-ethylhexoate.

#### References Cited in the file of this patent

##### UNITED STATES PATENTS

|    |           |                       |                |
|----|-----------|-----------------------|----------------|
| 40 | 2,001,108 | Parker -----          | May 14, 1935   |
|    | 2,345,580 | Buxton -----          | Apr. 4, 1944   |
|    | 2,363,722 | Faust -----           | Nov. 28, 1944  |
|    | 2,384,551 | Jehle -----           | Sept. 11, 1945 |
|    | 2,628,195 | Allison et al. -----  | Feb. 10, 1953  |
|    | 2,671,758 | Vinograd et al. ----- | Mar. 9, 1954   |